

Oct. 26, 1943.

A. UNGER

2,332,833

## TEXTILE MATERIAL AND METHOD OF MAKING

Filed Feb. 16, 1942



*INVENTOR.*

*Abraham Under*  
BY

Norman K. Holland  
ATTORNEY

## UNITED STATES PATENT OFFICE

2,332,833

TEXTILE MATERIAL AND METHOD OF  
MAKING

Abraham Unger, East Orange, N. J., assignor to  
Duro Persian Manufacturing Co., Inc., East  
Newark, N. J., a corporation of New Jersey

Application February 16, 1942, Serial No. 431,137

16 Claims. (Cl. 57—149)

The present invention relates to textiles and more particularly to textiles used in the manufacture of imitation Persian lamb cloth and to an improved method of making.

Imitation Persian lamb cloth has been manufactured by securing curled chenille to a suitable backing, the curled chenille being disposed on the backing in closely adjacent irregular rows to simulate the appearance of Persian lamb fur. Such cloth has been sold extensively, but its durability has been of such a limited nature as to deter repeat orders from customers. In use, the ends of the chenille fibers frequently lose their curl due to dampness and age. In addition, any rubbing tends to pull the loose ends of the fibers out and to mar the appearance of the cloth. For these reasons, the percentage of complaints by persons buying garments made from the cloth were sufficiently great that many stores discontinued the purchase of garments made from it. An attempt to overcome this objection has been made by utilizing wrapped cords instead of the curled chenille previously used. These wrapped cords presented difficulties which prevented the commercial manufacture and sale of cloth therefrom.

The present invention aims to overcome the above and other difficulties by providing an improved textile, made in part from a strand of chenille which has the advantage and appearance of curled chenille in the manufacture of Persian lamb fabrics and at the same time has satisfactory durability which cloth made from curled chenille does not have, whereby the manufactured cloth is satisfactory for sale as garments and will not impair customers' good will by failing to withstand the usual wear. The invention also provides an improved method of producing the article.

An object of the present invention is to provide an improved strand of textile material particularly useful in the manufacture of imitation Persian lamb cloth.

Another object of the invention is to provide an improved method of making a strand of textile material.

Another object of the invention is to provide an improved cloth having the appearance of Persian lamb fur.

Another object of the invention is to provide an improved strand of textile material which has substantially the softness and flexibility of curled chenille and which is more durable than curled chenille.

Another object of the invention is to enclose

the fibers of a strand of chenille to improve its durability without detracting from its appearance.

Other and further objects of the invention will be obvious upon an understanding of the illustrative embodiment about to be described, or will be indicated in the appended claims, and various advantages not referred to herein will occur to one skilled in the art upon employment of the invention in practice.

A preferred embodiment of the invention has been chosen for purposes of illustration and description and is shown in the accompanying drawing, forming a part of the specification, wherein

Fig. 1 is a sectional view illustrating the improved method and also illustrating the strand of material in its various stages leading to the finished form;

Fig. 2 is a sectional view along the line 2—2 of Fig. 1 illustrating the cut chenille as it appears before entering the tube;

Fig. 3 is a sectional view along the line 3—3 of Fig. 1 illustrating a section through a finished strand of the textile material;

Fig. 4 is a fragmentary top plan view of a piece of cloth made from the textile material to imitate Persian lamb fur;

Fig. 5 is an enlarged view of one coil of the textile material of the cloth;

Fig. 6 is a horizontal sectional view through the coil shown in Fig. 5; and

Fig. 7 is a sectional view through a modified form of the strand of textile material, illustrating the use of curled chenille for holding the outer wound casing in position.

For convenience, the method will be first described as the structural features of the strand of textile will be clear from its description. In the preferred method of making, illustrated in Figs. 1 to 3, a tube 1 is provided having a flared opening at its entrance end 2 which tapers down to a desired internal diameter at its outlet end 4. The exterior of the tube preferably tapers down also toward the outlet end to facilitate the application of the wound textile as will be described hereinafter. A strand of cut chenille 5 is passed through the interior of the tube 1. Cut chenille is known in the art and generally comprises a pair of twisted threads with outwardly projecting fibers of any desired length secured at their middle by the twisted threads. The appearance in side elevation is illustrated in Fig. 1 of the drawing before the chenille enters the tube and is illustrated in section in Fig. 2 of the

drawing. The radially projecting fibers 6 form, in effect, a cylindrical surface. As the strand of chenille 5 passes through the tube 1, the fibers 6 are bent backwardly as shown at 7 so that the external diameter is substantially less than before it entered the tube. The exterior of the tube has a thread 9 wound on it preferably by a holder (not shown) for a spool 8, which revolves around the tube continuously to apply the thread thereto. The exterior of the tube is preferably tapered so that the chenille thread 5 passing through the outlet end 4 of the tube engages the wrapped thread 9 and pulls it off of the end of the tube and carries it with the chenille. In this way, the exterior of the tube governs the size of the finished strand of material. The bent fibers 6 of the chenille tend to straighten and hence exert an outward pressure on the wrapped thread 9, tending to hold it in its outermost position and in substantially cylindrical form. The thread is preferably made of a series of strands which completely cover the exterior of the strand of chenille and form, in effect, a closed casing thereabout. The bent fibers of the chenille, in pressing outwardly, tend to hold the strands forming the casing in place and tend to prevent separation thereof and exposure of the enclosed fibers. When the strand of chenille is bent, the casing will have a tendency to slip on the enclosed strand of chenille and hence a chenille strand can be bent into flat turns, as illustrated in Fig. 5. Any separation of the strands 9 will not detract from the appearance or the durability of the finished cloth but actually produces irregularities which improves the appearance by making it resemble more nearly Persian lamb fur, which has numerous irregularities in it.

While the chenille may be formed of any suitable material, in the preferred form the fibers 6 are formed from sized or stiffened rayon or from visca straw, that is, artificial straw. It will be understood that good results may be had with other types of material; for example, wool, mohair, etc. Sized rayon and visca straw are stiff and tend to hold the wrapped textile 9 in place. At the same time, the outer casing formed by the wrapped textile 9 may be distorted in sewing and bending so that it resembles very closely Persian lamb fur. The appearance of the finished strand in section is illustrated in Fig. 3, where the bent fibers 7 are shown held in position by the textile wrapping 9. The fibers 6, in passing through the tube are bent backwardly so that they are bent down at an angle to the central axis of the strand of chenille.

It will be understood that the strands of textile material may be made in various sizes. Excellent results have been obtained by utilizing a tube having an internal diameter at its outlet end of one-eighth inch with a strand of cut chenille having a diameter of about one-quarter of an inch. The encased chenille formed was about nine thirty-seconds of an inch in diameter. The dimensions given are to be considered as illustrative only.

The strands of textile made in accordance with the method described above may be sewed to a backing 11 as illustrated in Fig. 4 by any suitable machinery. The composition of the strand is such that needles will readily pierce it and it may be sewed to the backing without encountering difficulties with sewing machinery. The stitches create irregularities in the surface of the outer casing and tend to give the appearance of Persian lamb fur. By reason of the texture of

the strand, it may be bent into a flat bend, as illustrated in Fig. 5, without causing the threads 9 to spread apart sufficiently to impair the article in any way. Preferably the threads are made up of a series of untwisted individual threads so that they spread over each other and tend to stay together. It will be noted from Fig. 4 that the appearance compares in all respects with imitation fur fabrics formed of curled chenille. At the same time, the threads 9 enclosing the strand of chenille prevent the fibers 6 from being materially exposed and hence it is able to withstand wear without giving a frazzled or worn look. The present fabric and the present strand of material for making it are a substantial improvement over a fabric made from curled chenille or a fabric made from wrapped cords.

A modified form of the invention is illustrated in Fig. 7, wherein curled chenille is used instead of the chenille illustrated in Figs. 1 to 3. In this case, a strand of curled chenille having curled or swirled fibers 6a and a core 12a is passed through the interior of the tube 1 and the wound textile 9a applied to it. The curled chenille will produce excellent results, but the uncurled chenille illustrated in the preferred embodiment is preferred.

It will be seen that the present invention provides an inexpensive imitation fur cloth having the appearance of Persian lamb. The cloth is durable and is adapted to give excellent wear under various weather and humidity conditions. The free ends of the chenille are substantially enclosed by a continuous textile thread wrapped about it, thereby greatly increasing the durability of the article without impairing its appearance. The use of the chenille, particularly chenille made of stiffened rayon or visca straw, affords a slight outward pressure tending to hold the outer casing in position and to prevent disarrangement of the thread wrapped thereabout. While the strand of material may have other uses, it is particularly useful in covering backing to form a cloth which simulates the appearance of Persian lamb fur. The cloth made as described herein is fully capable of withstanding the rough usage to which it may be subjected.

As various changes may be made in the form, construction and arrangement of the parts herein without departing from the spirit and scope of the invention and without sacrificing any of its advantages, it is to be understood that all matter herein is to be interpreted as illustrative and not in a limiting sense.

Having thus described my invention, I claim:

55. 1. The method of making an article of the class described, which comprises forming a strand of chenille having the outwardly extending fibers thereof inclined with respect to the axis of said strand, and placing a fibrous covering material over said strand so that the fibers of said latter material extend substantially transversely to the axis of the strand of chenille.
60. 2. The method of making a textile member, which method comprises passing a strand of material, having outwardly projecting bendable fibers, through a tube member to bend said fibers toward the axis thereof and applying a wound textile to said fibers, whereby the bent fibers tend to retain the wound textile in substantially cylindrical form.
65. 3. The method of making a textile member, which method comprises passing a strand of material, having outwardly projecting bendable fibers, through a tubular member, to bend said fibers toward the axis thereof, winding a textile

about the exterior of the tubular member and applying the wound textile to said bent fibers as they emerge from the end of the tubular member, whereby the bent fibers tend to retain the wound textile in substantially circular form.

4. The method of making a readily bendable textile member which method comprises forming a strand of material having fibers of substantial length projecting outwardly therefrom, bending said fibers toward the axis of the strand, and applying a textile winding to the bent fibers of the strand, whereby the bent fibers tend to force the textile winding into its outermost position.

5. The method of making an imitation Persian lamb cloth which method comprises forming a strand of material having fibers of substantial length projecting outwardly therefrom, bending said fibers toward the axis of the strand, applying a textile winding to the bent fibers of the strand, whereby the bent fibers tend to force the textile winding into its outermost position, and thereafter securing said encased strand of material to a backing in closely adjacent contorted rows thereon to simulate Persian lamb fur.

6. An article of manufacture comprising a strand of textile material having a wound exterior casing of non-rigid material, said strand of textile material having bent radially extending fibers pressing against the outer casing to hold it in its outer position.

7. An article of manufacture comprising a strand of textile material having an exterior casing and a strand of chenille within the casing with the outwardly extending fibers of the chenille held under compression by the outer casing.

8. An article of manufacture comprising a strand of textile material having a wound exterior casing and a strand of chenille within the casing, with the outwardly extending fibers of the chenille inclined toward the axis of the strand of chenille and held under compression by the outer casing.

9. An article of manufacture comprising a strand of textile material having a wound exterior casing and a strand of cut chenille within the casing, the outwardly extending fibers of the strand of the chenille being made of sized rayon and the outwardly extending rayon fibers being held under compression by the outer casing.

10. An article of manufacture comprising a strand of textile material having an exterior casing of non-rigid material and a strand of

chenille within the casing, having outwardly extending stiffened fibers, said stiffened fibers being bent out of their normally straight position by the outer casing, the tendency of said fibers to straighten exerting a force on the casing tending to hold it substantially in cylindrical form.

11. An article of manufacture comprising a strand of textile material having a wound exterior casing of non-rigid material and a strand of chenille within the casing with the fibers thereof curled to support the outer casing.

12. An article of manufacture comprising a strand of textile material having a wound exterior casing of non-rigid material and a strand of chenille within the casing with the fibers thereof bent to support the outer casing.

13. An imitation Persian lamb cloth comprising a backing, and a strand of textile material secured thereto in contorted outline to cover the backing, said strand of textile material comprising a strand of chenille having a wound exterior casing thereover of non-rigid material, the fibers of the chenille being bent to support the casing.

14. An imitation Persian lamb cloth comprising a backing, a strand of textile material secured thereto in a zigzag outline with substantially flat folds or bends therein to cover the backing, said strand of textile material comprising a strand of chenille having a wound exterior casing thereover of non-rigid material, said chenille permitting slippage of the casing thereon to facilitate sharp bends.

15. An imitation Persian lamb cloth comprising a backing, a strand of textile material secured to the backing in a series of adjacent rows with reverse bends therein to simulate Persian lamb, said strand of textile material comprising a strand of chenille having a wound exterior casing thereover of non-rigid material, the fibers of the strand of chenille being bent to support the casing, whereby said strand may be bent into flat folds and may be distorted to simulate Persian lamb.

16. An imitation Persian lamb cloth comprising a backing, a strand of textile material stitched thereto in a series of zigzag rows closely adjacent each other, with reverse bends in the material, to cover the backing, said strand of textile material comprising a strand of chenille having fibers made of stiffened rayon and having a substantially circular exterior casing thereover of a non-rigid material.

ABRAHAM UNGER.